

## UNITED STATES PATENT OFFICE

2,057,473

## SEMISOLID PLASTIC LUBRICANT

Eli F. Burch, Laurel Springs, N. J., assignor to  
 Cities Service Oil Company, Philadelphia, Pa.,  
 a corporation of Pennsylvania

No Drawing. Application June 20, 1935,  
 Serial No. 27,562

3 Claims. (Cl. 87—9)

This invention relates to lubricating compounds, and more particularly concerns an improved form of semi-solid plastic lubricant of the general type described in my recently expired U. S. Letters Patent No. 1,238,101, patented August 28th, 1917.

The primary object of the present invention is to provide a semi-solid plastic lubricant which shall be an improvement on the lubricant described in my aforementioned Patent No. 1,238,101; and which lubricant shall have a wider field of application in the lubrication of gears, shackle bolts, hydraulic machinery bearings, and as a blending agent for imparting to other lubricants such as soda base greases, valuable characteristics including water resistance and adhesive properties.

The improvement which forms the subject of the present invention developed from the discovery that by employing about 1 to 5% by weight of drying or semi-drying oil such as fish oil or linseed oil in compounding the lubricant, I can produce a lubricant of improved characteristics from a far wider range of basic ingredients than were suitable for use in preparing the lubricant which is described in my aforementioned Patent No. 1,238,101.

The general method of preparing the lubricant which forms the subject of the present invention does not differ markedly from that described in my aforementioned Patent No. 1,238,101. For example, I may take the heavy residual oil remaining after distillation of asphalt base crude petroleum such as produced in the South Texas field, without substantial cracking, and after separation of the light gasoline, kerosene and gas oil fractions; and admix with approximately 72% by weight of this residual oil about 25% by weight of No. 5 spindle oil or other light paraffinic lubricating oil, and approximately 3% by weight of commercial fish oil. These oils are mixed in a still at a temperature of approximately 200° F. and thoroughly agitated by blowing air therethrough while the temperature is raised to approximately 400° F. to 450° F. The air blowing of the mixture is continued at the temperatures specified for a period of 65 to 80 hours. The blowing operation is continued under heat until the mixture is reduced to a suitable semi-solid or grease consistency, for example, about as thick as hard Vaseline or commercial lubricating grease. I have found that I can prepare the lubricant in the above manner from almost any naphthenic base petroleum residuum, and that I also have a wide choice in proportioning the ingredients. Thus, I may employ 50 to 80 parts by weight of

the naphthenic base petroleum residuum, together with 45 to 15 parts by weight of light paraffinic petroleum lubricant, and 1 to 5 parts by weight of a drying or semi-drying oil having an iodine value in the range 125 to 175.

The resultant lubricant possesses a high degree of plasticity and has great affinity for metallic surfaces, is very unctuous and is stable in maintaining its consistency over a wide range of temperature. The lubricant is also characterized by having a low internal friction coefficient as compared to greases such as are compounded from soap and lubricating oils. The product is non-fluid at ordinary temperatures when left to stand, and slowly fluid when stirred, setting up again as a non-fluid when allowed to rest; thus the product is not adapted to viscosity measurements and is too fluid to be measured by the penetrometer except when it is set up, which condition does not measure the characteristics of the product which impart its commercial value.

I have found that the method which is described in my aforementioned Patent No. 1,238,101 is not applicable to the treatment of naphthenic base petroleum residua in general, whereas the improved process is broadly applicable and produces a satisfactory plastic lubricant. A suitable plastic lubricant prepared as described herein analyzed about 18% asphaltene content, and about 40% asphaltic resins. The product thus analyzed was found to contain 7-8% saponifiable material, although only 3% saponifiable oil (fish oil) was used in its preparation. The petroleum residuum which was used in preparing the lubricant above referred to had an asphaltene content of about 0.2%, and an asphaltic resin content of approximately 11%. Other suitable lubricants have been prepared from this same oil having an asphaltene content of 10% to 20%, and an asphaltic resin content in the range 35% to 45%. A microscopic examination of the product shows the asphalt particles are smooth and regular in outline, whereas the asphalt particles in the petroleum residuum are rough and irregular in outline. The fish oil or its oxidized product apparently acts as a protective colloid for the asphalt particles, preventing their agglomeration, and increasing their solubility in the oil-asphaltic resin matrix, so that the finished lubricant appears to comprise a smooth uniform dispersion of asphaltene particles in a mixture of mineral oil and asphaltic resins.

The invention having been thus described, what is claimed as new is:

1. A semi-solid plastic lubricant consisting es- 55

- sentially of a thoroughly oxidized and homogenized mixture of 50 to 80 parts by weight of naphthenic base petroleum residuum, 45 to 15 parts by weight of light paraffinic petroleum lubricant, and about 1 to 5 parts by weight of drying oil having an iodine value in the range 125-175, said lubricant being unctuous, insoluble in water, stable in consistency over a wide temperature range, possessing great affinity for metallic surfaces, and having a low friction coefficient as compared to soap grease.
2. A semi-solid plastic lubricant consisting essentially of a thoroughly oxidized and homogenized mixture of 50 to 80 parts by weight of naphthenic base petroleum oil residuum, about

45 to 15 parts by weight of spindle oil and about 1 to 3 parts by weight of fish oil.

3. The process of preparing a lubricant which consists in mixing about 50 to 80 parts by weight of naphthenic base petroleum oil residuum, about 45 to 15 parts by weight of spindle oil and about 1 to 5 parts by weight of a drying oil having an iodine value in the range of 125 to 175, heating the mixture to a temperature of approximately 400° F. to 450° F. and blowing air through the mixture at the temperatures specified for a period of 65 to 80 hours to reduce the mixture to a homogenized stable mass having a thick plastic consistency.

ELI F. BURCH. 15